

## UNITED STATES PATENT OFFICE

2,150,349

PROCESS AND PRODUCT RELATING TO  
ORGANIC METAL AND METALLOID CON-  
TAINING COMPLEX COMPOUNDS

Adrianus Johannes van Peski and Johannes Andreas van Melsen, Amsterdam, Netherlands, assignors to Shell Development Company, San Francisco, Calif., a corporation of Delaware

No Drawing. Application April 10, 1936, Serial No. 73,710. In the Netherlands April 11, 1935

15 Claims. (Cl. 260—438)

This invention relates to the production of valuable organic metal and metalloid-containing complex compounds, and it further relates to a novel class of organic metal and metalloid-containing complex compounds, which complex compounds are adaptable to a wide variety of purposes and which are particularly useful as means whereby metals in a soluble form can be introduced into hydrocarbons and particularly hydrocarbon fractions, such as motor fuels, natural and synthetic oils, lignite products, tar oils and the like, for the purpose of improving these materials.

Three main groups or classes of compounds are contemplated as reactants in accordance with the process of the invention. In a preferred embodiment of the invention one or more members selected from each of the classes of reactants hereinafter described is caused to react simultaneously with one or more members selected from each of the other two classes of reactants.

The first class of reactants, hereinafter designated as the "metal compounds", embraces the metal oxides, metal hydroxides and metal salts of weak acids.

The second class of reactants embraces organic compounds which possess one or a plurality of readily replaceable hydrogen atoms. The following are representative types of compounds contemplated as members of this class: the organic acids, the alcohols, the phenols, acid amides, amines, nitriles, aminoalcohols, phosphines, mercaptans, thioethers, the cyclodiolefins, acetylene, acetylene homologues, and the like.

The third class of reactants embraces the organic compounds of the elements of the right hand side of groups V and VI which have an atomic number not less than fifteen, and the organic compounds of the element nitrogen. A preferred subgroup of the compounds of this class includes the alkyl, aryl, aralkyl and cycloaliphatic compounds, as well as the substitution products thereof, of the metalloid elements phosphorus, arsenic, antimony, sulphur, selenium, tellurium and nitrogen and the organic esters of the acids of these metalloid elements.

The process of the invention comprises effecting the simultaneous reaction of a compound of the class consisting of metal oxides, metal hydroxides and metal salts of weak acids with an organic compound containing one or a plurality of readily replaceable hydrogen atoms and with an organic compound of an element of the right hand side of groups V and VI of the periodic table which has an atomic number not less than fifteen, and the element nitrogen, whereby an or-

ganic metal and metalloid-containing complex compound is formed.

A valuable feature of the present invention is inherent in the simultaneous reaction of a member of one of the classes of compounds with at least one member selected from each of the other two classes. In accordance with the process of the invention, the necessity of first preparing and isolating the organic metal compounds which it is desired to react with an organic metalloid compound to obtain a metal and metalloid-containing complex organic compound of a predetermined composition, is obviated. This is a very advantageous feature of the invention for the reason that many of the organic metal compounds, such as those which might be prepared by reacting a metal oxide, metal hydroxide or metal salt of a weak acid with an organic compound containing a readily replaceable hydrogen atom, are extremely difficult to prepare in practical yields and in some cases cannot be prepared at all, in still other cases the organic metal compounds may be so unstable as to render their use impractical and even dangerous. The advantages inherent in the present invention are clearly shown by the following example: In the case that it is desired to prepare organic metal compound complexes with an organic phosphine, for example, it is not always possible, or on account of the dangers and difficulties attendant thereon, desirable to prepare such organic metal and metalloid-containing complexes by first preparing the organic metal compound and subsequently reacting it with the organic phosphine or other organic metalloid compound. In many cases, the desired organic metal compound may be unavailable or it may be so unstable as to preclude its economical use. In accordance with the process of the present invention these difficulties are obviated and by a suitable selection of readily available reactants of the classes herein described any desired organic metal and metalloid-containing complex compound can be prepared economically in a practical yield.

As preferably employed specific members of the class of metal oxides, metal hydroxides and metal salts of weak acids, the following come into consideration: the alkali metal oxides, the alkali metal hydroxides, the alkaline earth metal oxides, the alkaline earth metal hydroxides, aluminum hydroxides, aluminum oxide, cuprous oxide, cupric oxide, cupric hydroxide, cuprous hydroxide, silver oxide, magnesium hydroxide, magnesium oxide, cadmium hydroxide, cadmium oxide, mercuric hydroxide, mercuric oxide, mercurous ox-

ide, thallium hydroxide, the thallium oxides, the zirconium oxides and hydroxides, the stannous and stannic oxides and hydroxides, the molybdenum oxides, lead hydroxide, the lead oxides, 5 thorium oxide, thorium hydroxide, the nickel oxides and hydroxides, the iron oxides and hydroxides, the cobalt oxides, the cobalt hydroxides, the noble metal oxides and hydroxides as the platinum hydroxides, the platinum oxides, palladium hydroxide, the gold hydroxides, the gold oxides, and the like. Suitable metal salts of weak acids include the alkali metal and alkaline earth metal carbonates and bicarbonates, copper carbonate, magnesium carbonate, the metal borates, 10 the metal tetraborates, the metal salts of the organic acids of which sodium formate, sodium acetate, copper formate, copper acetate, copper propionate, copper butyrate, lead acetate, nickel formate, nickel acetate, nickel oleate and the like 15 are representative.

Preferably, when metal salts of weak acids are used in the execution of the invention, the particular metal salt is selected with respect to the compound containing a readily replaceable hydrogen atom so that the compound in which the hydrogen atom is to be replaced by a metal atom has a stronger acid character than the weak acid from which the metal salt has been prepared.

The following compounds are representative 30 of organic compounds which contain at least one readily replaceable hydrogen atom: the organic monobasic and polybasic acids of saturated and unsaturated character as formic acid, acetic acid, propionic acid, butyric acid, isobutyric acid, the valeric acids and homologues and suitable substitution products of these aliphatic acids, benzoic acid, cinnamic acid, maleic acid, malonic acid, oxalic acid, lactic acid, succinic acid, the higher unsaturated acids as oleic, palmitic and the like; 35 the saturated and unsaturated alcohols of monohydric as well as polyhydric character as methyl alcohol, ethyl alcohol, the propyl alcohols, primary butyl alcohol, secondary butyl alcohol, tertiary butyl alcohol, the amyl alcohols and the like, ethylene glycol, propylene glycol, the butylene glycols, the amylene glycols, diethylene glycol, dipropylene glycol, the dibutylene glycols, triethylene glycol, tripropylene glycol, glycerol, di-glycerol,  $\beta$ -methyl glycerol, di- $\beta$ -methyl glycerol, 40 erythritol and the like and their homologues, analogues and suitable substitution products. The unsaturated alcohols as allyl alcohol, crotyl alcohol, isobutanol, cinnamyl alcohol, propargyl alcohol and the like are also suitable. Suitable phenolic bodies include phenol, the cresols, hydroquinone, pyrogallol, the naphthols, the xlenols and the like. Representative acid amides are formamide, ethanamide, propanamide, the butanamides, etc., and their homologues and analogues. The amines of primary, secondary and mixed character are suitable, the following being representative members: methyl amine, dimethyl amine, ethyl amine, diethyl amine, methyl ethyl amine, the propyl monoamines, the propyl di-amines, analine, phenylene diamine, ethylene diamine, and the like and their homologues and suitable substitution products. The nitriles are represented by the following aliphatic, aromatic and aralkyl compounds: aceto-nitrile, propio- 45 nitrile, butyro-nitrile, valero-nitrile, palmito-nitrile, methyl isocyanide, ethyl isocyanide, benzo-nitrile, benzyl cyanide and the like. Suitable amino-alcohols include the mono-, di- and tri-methanolamines, monoethanolamine, triethanolamine, diethanolamine, the mono- and poly-

propanol amines, methyl amino-propanol and the like and their homologues, analogues and suitable substitution products. Suitable phosphines include methyl phosphine, dimethyl phosphine, ethyl phosphine, diethyl phosphine, propyl phosphine, butyl phosphine, phenyl phosphine, benzyl phosphine and the like. Suitable mercaptans include the saturated and unsaturated alkyl and aralkyl mercaptans and the aromatic and other cyclic mercaptans as methyl mercaptan, ethyl mercaptan, the propyl mercaptans, allyl mercaptan, crotyl mercaptan, isobutetyl mercaptan, the butyl mercaptans, benzyl mercaptan, phenyl mercaptan and the like and their homologues. Suitable hydrocarbons which contain readily replaceable hydrogen atoms include, among others, the alkadienes, as butadiene, pentadiene, hexadiene, etc., and particularly the cycloalkadienes as cyclobutadiene, cyclopentadiene, cyclohexadiene, cycloheptadiene and the like and compounds containing an acetylenic linkage as acetylene and its homologues as methyl acetylene and the like and other suitable hydrocarbons containing readily replaceable hydrogen atoms.

Examples of suitable substituted and non-substituted alkyl, aralkyl, aryl and cycloaliphatic compounds of the elements of the right hand side of groups V and VI of the periodic table which have an atomic number not less than 15, and the element nitrogen and the esters of acids of these compounds, are pyridine, ethyl amine, ethyl diamine, ethyl triamine, the methyl, propyl, butyl and the higher amines, the mixed amines as ethyl propyl amine, aniline, ethylene diamine, phenylene diamine, ethanolamine, diethanolamine, triethanolamine, propanolamine, aminoacetic acid, aminobutyric acid, ethyl carbylamine, propyl carbylamine, phenyl carbylamine, aceto-nitrile, propio-nitrile, butyro-nitrile, trimethyl phosphine, triethyl phosphine, tripropyl phosphine, 40 tributyl phosphine, tribenzyl phosphine, triphenyl phosphine, trimethyl phosphite, triethyl phosphite, tripropyl phosphite, tributyl phosphite, trimethyl stibine, triethyl stibine, tripropyl stibine, tributyl stibine, methyl ethyl sulphide, dimethyl sulphide, diethyl sulphide, dipropyl sulphide, dibutyl sulphide, S-ethyl thioglycolic acid, ethyl ester, ethylene diethyl sulphide, propylene diethyl sulphide, diethyl disulphide, dimethyl selenium, diethyl selenium, dipropyl selenium, dibutyl 50 selenium, allyl sulphide, isobutetyl sulphide, dimethyl tellurium, trimethyl arsine, triethyl arsine, bismuth trimethyl, diethyl tellurium and the like and their homologues, analogues and suitable substitution products.

The reaction may be effected with any suitable proportion of the reactants depending upon the particular operation and the particular complex compound desired. In some cases it is desirable to execute the invention with the reactants present in the reaction mixture in equivalent amounts or with the other reactants in excess of the metal oxide, metal hydroxide or metal salt of a weak acid so as to facilitate conversion of the latter.

The reaction is preferably effected in a reaction vessel equipped with suitable heating and cooling means and means for agitating the reaction mixture as by shaking or mechanical stirring. The reactants may be introduced into the reaction vessel in any desirable manner and order provided that the reactants are present in the reaction mixture at such a time and in such amounts that simultaneous reaction of the three classes of reactants occurs. The reaction may be effected at any desired temperature and pres-

reaction time depends on sufficient time and to some extent on the reaction temperature. In some cases, the reaction takes place when the reactants are brought together in the desired proportions at about room temperature. In some cases, the temperature of the reaction mixture rises rapidly due to heat liberated during the course of the reaction. In such cases, the temperature of the reaction mixture can be controlled as desired, for example, by the use of external cooling means. If the reaction proceeds too slowly at room temperature or lower, it may be accelerated by the application of heat, by intensive stirring and/or other suitable means.

If desired the reaction can be effected in a relatively inert medium, which medium may act merely as a diluent and thus aid in control of the reaction or act as a solvent for one or more of the reactants and/or the reaction product or products. Suitable substantially inert diluents include among others the liquid hydrocarbons as benzol, hexylene, heptylene, octylene, octane, iso-octane, hydrocarbon fractions, mineral oils, shale oils and the like. The organic metal and metalloid-containing complexes are generally soluble in such hydrocarbon materials and they may be recovered therefrom by suitable means as extraction, evaporation, distillation, distillation under reduced pressure, etc.

In many cases it is desirable to effect reaction in the medium of the material to which it is desired to add the organic metal and metalloid-containing complex. Thus, instead of first preparing the organic complex compound and then adding it per se to the hydrocarbon material to be improved, the complex compound may be prepared directly in the hydrocarbon material by adding thereto the required amounts of the respective reactants and effecting reaction as herein described.

To prevent oxidation of the reagents and/or reaction product during the course of the reaction, oxygen is preferably excluded from the reaction vessel. This is readily accomplished by effecting the reaction in an atmosphere of a substantially inert material as nitrogen, hydrogen, hydrocarbon gases, and the like. Prior to introduction of the reactants into the reaction vessel, the latter may be flushed out with the inert gaseous material and maintained during the reaction under the desired pressure of said material. If desired, the inert gaseous material may be intermittently or continuously passed into the reaction vessel.

The invention is illustrated by the following examples. It is to be understood that these examples are for purposes of illustration only and that it is not our intention to limit the invention to the specific methods, reactants, proportion of reactants, products and conditions of these examples.

**EXAMPLE I**  
*Preparation of cuprobutyrate-diethyl sulphide*

( $\text{CuOOCC}_3\text{H}_7\text{C}_2\text{H}_5\text{S-C}_2\text{H}_5$ )

A mixture consisting of about 3.0 gm. (0.021 mol) of cuprous oxide, about 7.6 gm. (0.084 mol) of diethyl sulphide and about 3.7 gm. (0.042 mol) of butyric acid was charged to a suitable reaction vessel and shaken at room temperature under a nitrogen atmosphere for about 30 minutes. During the shaking the temperature of the reaction mixture was increased by a small amount due to the exothermicity of the reaction.

Subsequent to the above treatment, the mixture was refluxed for about 2 hours with about 30 c. c. of benzol. At the end of this time the mixture was filtered. It was found that 1.8

gm. of cuprous oxide were left on the filter, thus indicating that about 40% of the applied cuprous oxide had been reacted. The filtrate was evaporated under a reduced pressure at a temperature not greater than about 60° C. The residue, a viscous liquid weighing about 5.9 gm., was found to be the practically pure complex of the formula  $\text{CuOOCC}_3\text{H}_7\text{C}_2\text{H}_5\text{S-C}_2\text{H}_5$ . This compound is readily soluble in benzene and other aromatic hydrocarbons.

**EXAMPLE II**

*Preparation of cupriure-tri-normal propyl phosphite* ( $\text{CuNCONH}_2\cdot 2(\text{C}_3\text{H}_7\text{O})_3\text{P}$ )

About 15.7 gm. (0.076 mols) of tri-n-propyl phosphite were mixed with about 3.0 gm. (0.038 mols) of cupric oxide and about 2.3 gm. (0.038 mols) of urea and the mixture heated at about 130° C. in a nitrogen atmosphere for about 3 hours. As the reaction proceeded, the cupric oxide went into solution until substantially all of it was dissolved at the end of 3 hours of treatment. The reaction product obtained was a dark brown viscous liquid of which more than 10% was soluble in a gasoline fraction free of aromatic hydrocarbons.

**EXAMPLE III**

*Preparation of cuprophenolate-triethyl phosphine* ( $\text{CuOC}_6\text{H}_5\cdot 2(\text{C}_2\text{H}_5)_3\text{P}$ )

About 9.5 gm. of triethyl phosphine were shaken in a nitrogen atmosphere with about 2.9 gm. of cuprous oxide and about 3.8 gm. of phenol dissolved in about 20 c. c. of benzol, at room temperature. Due to the heat liberated in the course of the reaction, the temperature of the reaction mixture was raised to about 60° C. After the heat generation had practically ceased, the mixture was refluxed for about 30 minutes. At the end of this time the mixture was cooled and filtered. About 0.4 gm. of cuprous oxide were left on the filter.

The filtrate was evaporated under a reduced pressure. The residue consisted of about 14.2 gm. of a highly viscous, light brown liquid of the formula  $\text{CuOC}_6\text{H}_5\cdot 2(\text{C}_2\text{H}_5)_3\text{P}$ . This substance is very readily soluble in aromatic-free benzene and in other hydrocarbons and hydrocarbon fractions.

**EXAMPLE IV**

*Preparation of silver acetamide-tri-normal propyl phosphine* ( $\text{AgNHCOCH}_3\cdot 2(\text{C}_3\text{H}_7)_3\text{P}$ )

A mixture consisting of about 8.9 gm. of tri-n-propyl phosphine, 3.2 gm. of silver oxide, 1.6 gm. of acetamide and about 30 c. c. of benzol was charged to a suitable reaction vessel equipped with a reflux condenser and mechanical stirring means, placed under a nitrogen atmosphere, and stirred and heated at the boiling temperature of the reaction mixture for about 1 hour. At the end of this time the reaction mixture was cooled and filtered. About 0.4 gm. of silver oxide, a small part of which had been reduced to metallic silver, were filtered from the mixture.

The filtrate was evaporated under a reduced pressure at about room temperature. About 12.7 gm. of residue were obtained. Analysis showed this residue to be the substantially pure double compound of one mol of silver acetamide with two mols of tri-normal propyl phosphine. This compound is readily soluble in aromatic-free benzines and other hydrocarbon fractions.

**EXAMPLE V**

*Production of nickel formanilide-tri-normal propyl phosphite* ( $\text{NiC}_14\text{H}_14\text{O}_2\text{N}_2\cdot 2(\text{C}_3\text{H}_7\text{O})_3\text{P}$ )

About 13.5 gm. of tri-n-propyl phosphite were heated with about 3.0 gm. of nickel hydroxide and about 3.9 gm. of formaniline in a nitrogen atmosphere at a temperature of about 170° C. to 5 180° C. for about 3 hours. At the end of this time the mixture was added to 1 liter of a benzine substantially free of aromatic hydrocarbons and the mixture shaken for about 12 hours. The mixture was then filtered and the filtrate analyzed. It contained more than 0.2% of Ni, bound in a double compound of the formula



#### EXAMPLE VI

15 *Preparation of cupro-cyclopentadiene-tri-normal propyl phosphine (CuC<sub>5</sub>H<sub>5</sub>.2(C<sub>3</sub>H<sub>7</sub>)<sub>3</sub>P)*

A mixture consisting of about 29 gm. of tri-n-propyl phosphine, about 6.5 gm. of cuprous oxide, about 6.0 gm. of cyclopentadiene and about 20 c. c. of benzol was charged to a suitable reaction vessel, put under a nitrogen atmosphere, and heated to the boiling temperature of the mixture for about 2 hours. A clearly perceptible reaction took place, as indicated by water formation 20 and the gradual consumption of the solid cuprous oxide. At the end of two hours of treatment the mixture was cooled and filtered. About 2.5 gm. of unreacted cuprous oxide were filtered from the mixture. The filtrate was evaporated to remove 25 the lower boiling constituents. The residue, about 34.4 gm. being obtained, was found to have the formula CuC<sub>5</sub>H<sub>5</sub>.2(C<sub>3</sub>H<sub>7</sub>)<sub>3</sub>P. This complex organic metal compound is readily soluble in benzine fractions, particularly in those fractions 30 substantially free of aromatics.

Other representative examples of valuable organic metal and metalloid complex compounds, which may be readily prepared in good yield in accordance with the process of our invention, are 40 the following:

|                                                     |                                                                                                                                 |
|-----------------------------------------------------|---------------------------------------------------------------------------------------------------------------------------------|
| Cupro-acetate-ethylene diamine.....                 | CuOOCCH <sub>3</sub> .C <sub>2</sub> H <sub>4</sub> (NH <sub>2</sub> ) <sub>2</sub>                                             |
| Cupro-urea-triethyl phosphine.....                  | CuNHCONH <sub>2</sub> .(C <sub>2</sub> H <sub>5</sub> ) <sub>3</sub> P                                                          |
| DiCupro-urea-triethyl phosphine.....                | Cu <sub>2</sub> NCONH <sub>2</sub> .(C <sub>2</sub> H <sub>5</sub> ) <sub>3</sub> P                                             |
| Cupro-phenolate-triethyl phosphite.....             | CuOC <sub>6</sub> H <sub>5</sub> .(C <sub>2</sub> H <sub>5</sub> ) <sub>3</sub> P                                               |
| Silver acetamide-triethyl phosphite.....            | AgNHOCC <sub>2</sub> H <sub>5</sub> .(C <sub>2</sub> H <sub>5</sub> ) <sub>3</sub> P                                            |
| 45 Cupro-cuprate-diethyl sulphide.....              | CuOOCCH <sub>3</sub> H <sub>7</sub> .(C <sub>2</sub> H <sub>5</sub> ) <sub>2</sub> S                                            |
| Cupro-butadiene-tripropyl phosphite.....            | CuC <sub>4</sub> H <sub>9</sub> .(C <sub>2</sub> H <sub>5</sub> ) <sub>3</sub> P                                                |
| Cupro-aniline-triethyl phosphite.....               | CuHNC <sub>6</sub> H <sub>5</sub> .(C <sub>2</sub> H <sub>5</sub> ) <sub>3</sub> P                                              |
| Nickel formamide-triethyl phosphite.....            | Ni(NHOCH <sub>2</sub> ) <sub>2</sub> .(C <sub>2</sub> H <sub>5</sub> ) <sub>3</sub> P                                           |
| Cupro-butyrate-ethylene diethyl sul-40 phide.....   | CuOOCCH <sub>3</sub> H <sub>7</sub> .C <sub>2</sub> H <sub>5</sub> (SC <sub>2</sub> H <sub>5</sub> ) <sub>2</sub>               |
| Cupro-propyl mercaptide - triheptyl phosphite.....  | CuSC <sub>6</sub> H <sub>5</sub> .(C <sub>7</sub> H <sub>15</sub> O) <sub>3</sub> P                                             |
| 50 Gold cyanide-triethyl phosphine.....             | AuCN.(C <sub>2</sub> H <sub>5</sub> ) <sub>3</sub> P                                                                            |
| Cobalt-phenolate-triethyl phosphine.....            | Co(O <sub>2</sub> C <sub>6</sub> H <sub>5</sub> ) <sub>3</sub> .(C <sub>2</sub> H <sub>5</sub> ) <sub>3</sub> P                 |
| Cobalt - formanilide - tripropyl phos-55 phite..... | CoC <sub>11</sub> H <sub>21</sub> O <sub>2</sub> N <sub>3</sub> .(C <sub>2</sub> H <sub>5</sub> ) <sub>3</sub> P                |
| Stanno-cresolate-triethyl phosphite.....            | Sn(O <sub>2</sub> C <sub>6</sub> H <sub>5</sub> CH <sub>3</sub> ) <sub>2</sub> .(C <sub>2</sub> H <sub>5</sub> ) <sub>3</sub> P |
| Ferric-phenolate-triethyl phosphite.....            | Fe(O <sub>2</sub> C <sub>6</sub> H <sub>5</sub> ) <sub>3</sub> .(C <sub>2</sub> H <sub>5</sub> ) <sub>3</sub> P                 |

55 When a compound of the class consisting of metal oxides, metal hydroxides and salts of weak acids is simultaneously reacted with a compound of the class consisting of alcohols, acid amides, amines, nitriles, aminoalcohols, phosphines, mercaptans, alkadienes, cycloalkadienes, acetylene and acetylene homologues and with an organic metalloid compound of the class consisting of the hydrocarbon and substituted hydrocarbon compounds of the elements of the right hand side 60 of groups V and VI of the periodic table which have an atomic number not less than 15, and the element nitrogen, and the organic esters of acids of these elements, the resulting organic metal and metalloid-containing complex compounds 65 are novel.

The members of this novel class of organic metal and metalloid-containing complex compounds may be represented by the general formula (MR).xZ, wherein (MR) represents the 70 compound of a metal with an organic compound

of the class consisting of alcohols, acid amides, amines, nitriles, aminoalcohols, phosphines, mercaptans, alkadienes, cycloalkadienes, acetylene and acetylene homologues, and Z represents an organic metalloid compound of the class consisting of the hydrocarbon and substituted hydrocarbon compounds of, and the organic esters of acids of, the elements of the right hand side of groups V and VI of the periodic table which have an atomic number not less than 15, and the element nitrogen, x representing an integer not usually greater than 2.

A valuable subgroup of novel organic metal and metalloid-containing complex compounds 15 embraces the double compounds of metal salts of organic acids and phenolic compounds with substituted or non-substituted alkyl, aralkyl, aryl and cycloaliphatic compounds of phosphorus, arsenic, 20 antimony, sulphur, selenium and tellurium or with organic esters of acids of these elements.

Another subgroup of novel organic metal and metalloid-containing complex compounds embraces the double compounds of inorganic metal salts, exclusive of the metal halides, with substituted or non-substituted alkyl, aralkyl, aryl and cycloaliphatic compounds of phosphorus, arsenic, 25 antimony, sulphur, selenium and tellurium or with organic esters of acids of these elements.

The organic metal and metalloid-containing 30 complex compounds are useful for a wide variety of purposes. They are of particular value as means of introducing metals in a soluble and active form into hydrocarbons and hydrocarbon mixtures, particularly motor fuels and lubricating oil compositions for the purpose of enhancing the value of such hydrocarbon materials and making them more suitable for special purposes.

The great majority of the organic complex 35 compounds which are prepared in accordance with the process of the invention are readily soluble to a considerable extent in a wide variety of organic solvents. They are even readily soluble in the non-polar and slightly polar solvents such as tar oil products (benzol and its homologues), petroleum fractions as kerosene, gasoline, gasoil, lubricating oils and the like, hydrogenation products of olefine polymers, coal, tar, mineral oils, shale oils, etc., cracking products of tars, waxes, mineral oils, animal oils, vegetable oils and the like carbonaceous materials. Consequently, the organic metal and metalloid-containing complex compounds may be dissolved in the required amount in a hydrocarbon material, or suspended in such a hydrocarbon material, to improve it in some desired respect. Many of the organic metal complex compounds when added to motor fuels as gasoline, iso-octane, etc., 50 improve the anti-knock properties of the fuels or fuel mixtures. The organic metal complex compounds also act as anti-oxidants, and when added to lubricating oils and greases render them suitable as extreme pressure lubricants.

While we have in the foregoing described in 55 some detail the preferred embodiment of our invention and some variants thereof, it will be understood that this is only for the purpose of making the invention more clear and that the same is not to be regarded as limited to the 60 details of operation described nor is it dependent upon the soundness or accuracy of the theories which we have advanced as to the advantageous results attained. On the other hand, the invention is to be regarded as limited only by the terms 70 75

of the appended claims, in which it is our intention to claim the invention as broadly as possible in view of the prior art.

We claim as our invention:

- 5 1. A process for the production of useful metal and metalloid-containing complex organic compounds which comprises bringing together and simultaneously reacting at least three different reactants, one reactant being a metal compound 10 of the class consisting of the metal oxides and metal hydroxides, another reactant being an organic compound containing a readily replaceable hydrogen atom but devoid of any acid-forming multivalent element of groups V and VI 15 of the periodic table which has an atomicity greater than one and an atomic number not greater than 52, and the third reactant being an organic compound of an acid-forming multivalent element of groups V and VI of the periodic 20 table which has an atomicity greater than one and an atomic number not greater than 52.
2. A process for the production of useful metal and metalloid-containing complex organic compounds which comprises bringing together and 25 simultaneously reacting, in the liquid phase, and in the presence of a substantially inert normally liquid diluent material, at least three different reactants, one reactant being a metal compound of the class consisting of the metal oxides and 30 metal hydroxides, another reactant being an organic compound containing a readily replaceable hydrogen atom but devoid of any acid-forming multivalent element of groups V and VI of the periodic table which has an atomicity greater than one and an atomic 35 number not greater than 52, and the third reactant being an organic compound of an acid-forming multivalent element of groups V and VI of the periodic table which has an atomicity greater than one and an atomic 40 number not greater than 52.
3. A process for the production of useful metal and metalloid-containing complex organic compounds which comprises bringing together and simultaneously reacting at least three different reactants, one reactant being a metal oxide, another reactant being an organic compound containing a readily replaceable hydrogen atom but devoid of any acid-forming multivalent element of groups V and VI of the periodic table which has an atomicity greater than one and an atomic 45 number not greater than 52, and the third reactant being an organic compound of an acid-forming multivalent element of groups V and VI of the periodic table which has an atomicity greater than one and an atomic 50 number not greater than 52.
4. A process for the production of a useful copper and metalloid-containing complex organic compound which comprises bringing together and simultaneously reacting at least three different reactants, one reactant being a copper oxide, another reactant being an organic compound containing a readily replaceable hydrogen atom but 55 devoid of any acid-forming multivalent element of groups V and VI of the periodic table which has an atomicity greater than one and an atomic number not greater than 52, and the third reactant being an organic compound of an acid-forming multivalent element of groups V and VI of the periodic table which has an atomicity greater than one and an atomic number not greater than 52.
5. A process for the production of useful metal 60 and metalloid-containing complex organic com-

pounds which comprises bringing together and simultaneously reacting at least three different reactants, one reactant being a metal compound of the class consisting of the metal oxides and metal hydroxides, another reactant being an organic hydroxy compound but devoid of any acid-forming multivalent element of groups V and VI of the periodic table which has an atomicity greater than one and an atomic number not greater than 52, and the third reactant being an organic compound of an acid-forming multivalent element of groups V and VI of the periodic table which has an atomicity greater than one and an atomic number not greater than 52.

6. A process for the production of useful metal and metalloid-containing complex organic compounds which comprises bringing together and simultaneously reacting at least three different reactants, one reactant being a metal compound of the class consisting of the metal oxides and metal hydroxides, another reactant being an organic compound containing a readily replaceable hydrogen atom but devoid of any acid-forming multivalent element of groups V and VI of the periodic table which has an atomicity greater than one and an atomic number not greater than 52, and the third reactant being an organic compound of the class consisting of the alkyl, aralkyl and aryl compounds of acid-forming multivalent elements of groups V and VI of the periodic table which have an atomicity greater than one and an atomic number not greater than 52.

7. A process for the production of useful metal and metalloid-containing complex organic compounds which comprises bringing together and simultaneously reacting at least three different reactants, one reactant being a metal compound of the class consisting of the metal oxides and metal hydroxides, another reactant being an organic compound containing a readily replaceable hydrogen atom but devoid of any acid-forming multivalent element of groups V and VI of the periodic table which has an atomicity greater than one and an atomic number not greater than 52, and the third reactant being an organic compound of the class consisting of the alkyl compound of an acid-forming multivalent element of groups V and VI of the periodic table which has an atomicity greater than one and an atomic number not greater than 52.

8. A process for the production of useful metal and metalloid-containing complex organic compounds which comprises bringing together and simultaneously reacting at least three different reactants, one reactant being a metal compound of the class consisting of the metal oxides and metal hydroxides, another reactant being an organic compound containing a readily replaceable hydrogen atom, and the third reactant being an alkyl ester of an inorganic acid of an acid-forming multivalent element of groups V and VI of the periodic table which has an atomicity greater than one and an atomic number not greater than 52.

9. A process for the production of useful metal and metalloid-containing complex organic compound which comprises bringing together and simultaneously reacting at least three different reactants, one reactant being a metal compound of the class consisting of the metal oxides and metal hydroxides, another reactant being an organic compound containing a readily replaceable hydrogen atom but devoid of phosphorus, and the third reactant being an organic compound of phosphorus.

10. A process for the production of cupro-butyrate-diethyl sulphide of the formula



- 5 which comprises reacting cuprous oxide simultaneously with butyric acid and with diethyl sulphide, the reaction being effected in the liquid phase in a substantially inert non-oxidizing atmosphere.
- 10 11. The metal and metalloid-containing complex organic compounds of the general formula (MR). $xZ$ , the group MR representing an organic compound wherein a readily replaceable hydrogen atom has been replaced by a metal radical, Z representing an organic compound of an acid-forming multivalent element of groups V and VI of the periodic table which has an atomicity greater than one and an atomic number not greater than 52, and  $x$  representing an integer not greater than two, the compound Z being bound to the group MR to form a metal-containing complex organic compound.
- 15 12. The metal and metalloid-containing complex organic compounds of the general formula (MR). $xZ$ , the group MR representing the metal salt of an organic acid, Z representing an organic compound of an acid-forming multivalent element of groups V and VI of the periodic table which has an atomicity greater than one and an atomic number not greater than 52, and  $x$  repre-

senting an integer not greater than two, the compound Z being bound to the group MR to form a metal-containing complex organic compound.

13. The complex compound: cupro-butyrate-diethyl sulphide of the formula



14. The copper-containing complex organic compound of the general formula (MR). $xZ$ , wherein MR represents the copper salt of a carboxylic acid,  $x$  represents an integer not greater than two, and Z represents an alkyl compound of an acid-forming multivalent element of groups V and VI of the periodic table which has an atomicity greater than one and an atomic number not greater than 52, Z being bound to MR to form a copper-containing complex organic compound.

15. The metal and metalloid-containing complex organic compound of the general formula (MR). $xZ$ , the group MR representing an organic compound devoid of phosphorus and wherein a readily replaceable hydrogen atom has been replaced by a metal radical, X representing an integer not greater than two and Z representing an organic compound of phosphorus, the compound Z being bound to the group MR to form a metal-containing complex organic compound.

ADRIANUS JOHANNES VAN PESKI.  
JOHANNES ANDREAS VAN MELSEN.

30